

Aug. 9, 1932.

R. GILLIS

1,871,317

MAGNETIC CORE AND METHOD OF MAKING THE SAME

Filed Sept. 10, 1930



Fig. 1.



Fig. 2.

Fig. 3.



Inventor  
R. Gillis

By H. B. Whisfield Atty.

## UNITED STATES PATENT OFFICE

RANDALL GILLIS, OF LA GRANGE, ILLINOIS, ASSIGNOR TO WESTERN ELECTRIC COMPANY, INCORPORATED, OF NEW YORK, N. Y., A CORPORATION OF NEW YORK

## MAGNETIC CORE AND METHOD OF MAKING THE SAME

Application filed September 10, 1930. Serial No. 480,880.

This invention relates to magnetic cores and methods of making the same, and more particularly to magnetic cores for loading coils used in telephone systems, and to methods of making such cores.

In general terms, the invention relates to the production of magnetic cores of the type disclosed in Patents 1,669,643 and 1,669,645 to J. W. Andrews et al., wherein finely divided particles of a magnetic material such as an alloy of nickel and iron are coated with an insulating material, and are then compressed into cores of the desired shape and size, which are heat treated to impart the desired electrical and magnetic properties thereto.

Objects of the invention are to provide cores having improved magnetic characteristics and lower hysteresis losses, and to provide an improved method of making such cores.

20 In accordance with one embodiment of the invention, a pressure materially higher than those heretofore used is employed in compressing the material into cores, and the cores are then subjected to an annealing treatment 25 to bring about the optimum of mechanical, electrical, and magnetic properties in the finished cores.

The invention will be clearly understood from the following detailed description of 30 one embodiment thereof, taken in connection with the accompanying drawing, in which

Fig. 1 is a graphical illustration showing the relation between the forming pressure and the hysteresis loss in magnetic cores;

35 Fig. 2 is a similar illustration showing the relation between the forming pressure and the permeability in magnetic cores, and

Fig. 3 is a perspective view of a section of 40 a loading coil core made in accordance with the present invention.

In carrying out the present invention the magnetic material employed is preferably prepared from a nickel-iron alloy known as permalloy, a ratio of 81 parts nickel to 19 parts iron being satisfactory for most purposes. The alloy is treated in the manner disclosed in Patent 1,669,649, issued May 15, 1928 to C. P. Beath et al. to reduce it to a finely divided form, the particles being preferably of

50 such fineness that they will pass a 120-mesh

screen or finer. The alloy particles are then annealed in the known manner, after which they are coated with an insulating material which insulates the particles from each other and which may be of the composition described in the J. W. Andrews et al. patents referred to above. The mass is then dried and pressed into cores or rings under sufficient pressure to create an autogenous bond between the insulated particles of metal which holds them together in rigid relation to each other.

In forming the mass into cores, it has been found that a pressure substantially in excess of 200,000 pounds per square inch is desirable in that the hysteresis loss in cores formed at such higher pressures is reduced. This may be seen from an examination of Fig. 1, wherein the abscissæ represent forming pressures in pounds per square inch and the ordinates represent hysteresis loss in watts per cycle per  $\text{cm}^2 \times 10^{10}$ . From the values shown in Fig. 1 and from further experiments it has been determined that a forming pressure of about 250,000 pounds per square inch or higher is especially suitable. The hysteresis loss of permalloy and other magnetic metals was thought to be increased by cold working but as evidenced by the curve in Fig. 1 a lower hysteresis loss is obtained by using higher forming pressures. It is believed that the decrease in hysteresis loss with increased forming pressure is due to the magnetic flux being more uniformly distributed throughout the cross-section of the core because of the core being more dense and homogeneous.

70 In a core formed at low pressure the particles of permalloy dust are more widely separated and although the flux per unit of cross-sectional area remains the same as for the highly compressed core, the flux 75 is concentrated in the particles of dust, thereby increasing the flux density within the particles themselves, and since the hysteresis loss is proportional to the 2.7 power of the flux density, it decreases with an increase in density or compactness of the core material.

It has also been found that the permeability of the cores increases with increased form-

ing pressure, as shown in Fig. 2, wherein the abscissæ represent forming pressure and the ordinates represent permeability in watts per cycle per  $\text{cm}^2 \times 10^{10}$ . It will be seen from 5 an examination of Fig. 2 that the permeability increases slowly but yet appreciably as the forming pressure is increased above 200,000 pounds per square inch. In other words, the property of permeability is not 10 adversely affected by the higher pressures, but on the contrary tends to slightly higher values.

After the cores have been compressed as above described, they may be annealed in the 15 known manner to impart the desired electrical and mechanical properties thereto, after which they are ready to receive the usual toroidal winding preparatory to being placed in a telephone system.

20 While the invention has been described in connection with a composition having certain specified ingredients, it is applicable to differently constituted compositions, and the details hereinabove set forth may be considerably varied without departing from the scope 25 of the invention.

What is claimed is:

1. A magnetic core composed of insulated particles of a nickel-iron alloy held together 30 by an autogenous bond formed under a pressure of about 250,000 pounds per square inch.
2. A method of forming magnetic cores from insulated particles of a nickel-iron alloy, which consists in compressing the particles 35 into the desired form under a pressure of about 250,000 pounds per square inch.
3. A method of forming magnetic cores from particles of a nickel-iron alloy, which consists in coating said particles with an insulating composition, compressing the insulated particles into a core under a pressure of 40 at least 250,000 pounds per square inch, and annealing the formed cores.

In witness whereof, I hereunto subscribe 45 my name this 29th day of August A. D., 1930.

RANDALL GILLIS.